

June 16, 1953

J. W. HORNE ET AL

2,642,380

RECOVERY OF WAXES FROM SHALE OIL

Filed July 5, 1951



INVENTORS

Joseph W. Horne

Peter R. Tisot

BY *Joseph W. Horne*

ATTORNEY

## UNITED STATES PATENT OFFICE

2,642,380

## RECOVERY OF WAXES FROM SHALE OIL

Joseph W. Horne and Peter R. Tisot, Laramie,  
Wyo., assignors to the United States of America  
as represented by the Secretary of the Interior

Application July 5, 1951, Serial No. 235,354

8 Claims. (Cl. 196—18)

(Granted under Title 35, U. S. Code (1952),  
sec. 266)

1

The invention herein described and claimed may be manufactured and used by or for the Government of the United States of America for governmental purposes without the payment of royalties thereon or therefor.

This invention relates to the recovery of olefinic and paraffinic waxes from shale oil.

The occurrence of waxy material in oil produced by the pyrolytic decomposition of the organic material (kerogen) contained in oil shale is, of course, well known. Up to the present time however, there has been relatively little investigation of these shale oil waxes, particularly in this country, and it has long been considered that these waxes, particularly those of higher melting point, are, like petroleum waxes, substantially paraffinic in character. Thus, it has been considered that the same methods employed for the recovery and purification of petroleum waxes, such as sweating or solvent extraction followed by acid treatment, would be equally applicable for separation and recovery of shale oil waxes.

It has been found, however, that in contrast to the waxes that may be obtained from petroleum, relatively high melting point waxes containing a high degree of olefinic unsaturation, as well as a fully paraffinic wax may be obtained from certain high boiling shale oil fractions. More specifically, it has been found that by solvent extracting a shale oil distillation fraction boiling between 675° and 950° F. to recover the waxy material contained therein and then separating, preferably by selective adsorption, the olefinic content of the waxy material from the paraffinic portion thereof, it is possible to produce one wax which is substantially paraffinic in nature, and another wax which is highly olefinic. The paraffinic wax produced in this manner will find application wherever high grade paraffin waxes are employed, such as in the food packaging industry. The olefinic wax produced in accordance with the invention is unique in that it is relatively high melting and of high molecular weight and yet contains a high percentage of olefinic unsaturation.

The crude oil which forms the source material for the production of waxes in accordance with the invention is obtained by the destructive distillation of naturally occurring oil shale at temperatures which usually range from 900° to 1300° F. In conformity with usage in the United States, the term "oil shale" in the specification and claims is intended to refer to

2

sedimentary rocks containing kerogen, regardless of their common or scientific designations, which upon destructive distillation yield a mixture of hydrocarbons and certain nitrogen and phenolic compounds, usually called "shale oil." Extensive deposits of oil shale are found in this country, particularly in Colorado, Utah, and Wyoming, and deposits of varying extent and richness are found in other countries throughout the world. The crude oils obtained by destructive distillation of domestic oil shale, particularly of the type found in Colorado, Wyoming, and Utah are particularly useful as source materials in connection with the present invention.

From the crude shale oil a distillation fraction is prepared, hereafter referred to as the wax distillate, boiling between 675° and 950° F. and preferably between 750° and 925° F. This wax distillate characteristically contains a high percentage of nitrogen compounds (in the case of Colorado shale oils from 35% to 50%) as well as a higher proportion of aromatic sulfur and oxygen compounds than are found in petroleum crudes. Separation of these nitrogen, aromatic, sulfur, and oxygen compounds, as well as the paraffin oils, from the hydrocarbon waxes is accomplished by extracting the wax distillate with a solvent which has strong solvent power for these components, but substantially no solvent power for the hydrocarbon waxes at the selected dewaxing temperature. A single solvent may be employed or if desired a blend of solvents. Methyl ethyl ketone used alone is highly satisfactory from the standpoint of the size and structure of the wax crystals produced, quantity of solvent required, filtration rate, quantity of wax recovered and the oil content of the wax extracted. A mixture of ethylene dichloride and acetone is also very satisfactory. Usually the wax distillate and the solvent or blend of solvents, are mixed thoroughly at a temperature sufficiently high to form a homogeneous solution and then the mixture chilled to crystallize out the wax. However, if desired, the wax distillate and solvent may be chilled separately to the dewaxing temperature and then thoroughly mixed.

At the dewaxing temperature, which preferably is in the range of 0° to 35° F., depending upon the solvent employed, and the melting point of the wax desired, the wax crystals separate from the mother liquor and are then filtered and washed. The filtrate or raffinate contains the oily material, including the nitro-

gen, aromatic, sulfur, and oxygen compounds present in the wax distillate.

The crude wax obtained in this manner is a hydrocarbon wax of relatively high melting point, usually ranging between 90° and 200° F., and in many respects resembles petroleum paraffin wax with the exception that it contains a relatively high percentage of olefinic unsaturation, usually from 15% to 18% by weight. If this mixture of olefinic and paraffinic waxes is refined by acid treatment in the usual manner of refining petroleum paraffin waxes, loss of the entire olefinic content of the wax would result with the consumption of a large amount of acid.

In accordance with the invention, instead of eliminating the olefin content by such methods as acid treating, the paraffinic and olefinic waxes contained in this mixture are separated from one another, preferably by selective adsorption, to produce two distinct waxes, one a paraffin wax, containing no olefinic unsaturation, and the other a relatively high melting point wax containing a high degree of olefinic unsaturation.

The following example illustrates the recovery of paraffinic and olefinic waxes from a shale oil produced by the destructive distillation of a domestic oil shale. For the purposes of clarity, reference will be made to the accompanying drawing which diagrammatically illustrates the procedure employed in this example. The wax distillate employed as the starting material in this example was obtained by fractionating a crude shale oil produced by retorting Colorado oil shale assaying about 30 gallons of crude oil per ton of shale by the so-called N-T-U retorting process. In accordance with this retorting process, crushed shale is loaded into a cylindrical retort and the shale at the top of the retort is then ignited and air is blown downwardly through the shale bed. Heat furnished by combustion of the upper layer of shale serves to decompose the kerogen in the layers of shale beneath the combustion zone. The oil vapors which distill from the shale are carried out in the retort in the hot gas stream. The combustion zone advances downwardly through the complete charge in the cylindrical retort, residual carbon in the shale from which the oil has already been driven supporting the combustion and furnishing heat throughout the retorting process. Distillation temperatures are in the neighborhood of from 850° to 1000° F.

The crude shale oil obtained in this manner was topped to 675° F. at 585 mm. of mercury. From the remaining bottoms, the wax distillate was continuously distilled at an overhead temperature of 525° F. (plus or minus 5° F.) at 5 mm. Hg (corresponding to 895° F. at 760 mm. Hg). The wax distillate constituted 35% of the crude oil.

Referring now to the drawing, the wax distillate in storage tank 1 was mixed in tank 3 with methylethyl ketone from solvent storage tank 2. The ratio of oil to solvent was 1:2 by volume. The oil-solvent mixture was warmed to effect complete solution of the crystallized wax, and was then transferred to chilling vessel 4 where it was chilled to 32° F. at the rate of 3° to 5° F. per hour. The wax which separated on cooling consisted of well defined plate crystals.

The mixture was next transferred to a filter 5 where the wax crystals were filtered off and washed with chilled solvent from wash solvent tank 6 to remove the oil adhering thereto. The filtrate containing the paraffin oils and the

aromatic and nitrogen compounds was transferred to stripping column 7 wherein the solvent was stripped from the dewaxed oil, condensed in condenser 8 and recycled to solvent storage tank 2 for reuse.

The wax removed from filter 5 had a flaky crystal structure, a light amber color, and an oil content of 0.10% to 0.20% by weight. This single-solvent extracted wax had the following composition:

|                          | Per cent |
|--------------------------|----------|
| Paraffins and naphthenes | 83.3     |
| Olefins                  | 16.7     |
| Aromatics                | 0.0      |

If desired, the single solvent extracted wax may be subjected to further solvent extraction to improve the color and further reduce the oil content. However this is not necessary since with a single solvent extraction, the oil content was reduced to within the limits ordinarily required of a fully refined petroleum paraffin wax.

The single solvent extracted wax was transferred to a steam deodorizer 9 where the crude wax was melted and agitated with wet steam to remove volatile odor-forming impurities. Condensed steam was separated from the wax in settling tank 10. After this treatment, the wax had no objectional odor or taste, had an amber color and contained the olefins present in the solvent extracted wax. This product remained color stable.

The steam treated wax was next transferred to a decolorizing tower 11 where it was decolorized by percolation through a bed of an activated bauxite (sold under the trade name Florite) sized to 20-60 mesh. By percolating the wax through the bauxite at 145° to 150° F. (about 15° F. above its melting point) with a contact time of about 5 hours, a water white product was obtained. The finished product was colorless, odorless, and tasteless, and had the following analysis:

|                          | Per cent |
|--------------------------|----------|
| Paraffins and naphthenes | 87.4     |
| Olefins                  | 12.6     |
| Aromatics                | 0.0      |

As will be noted, some of the olefins were adsorbed on the bauxite, resulting in a lower percentage of olefins in the refined paraffin-olefin wax. The olefins adsorbed during the decolorization treatment may be desorbed from the bauxite by a suitable eluent such as cyclohexanol, and if desired subjected to further purification.

The steam and bauxite-treated wax was then transferred to a melting tank 12 and the melted wax percolated through a tower 12 packed with silica gel adsorbent. Percolation was continued until the adsorption capacity of the silica gel column for the olefinic content of the mixed waxes was reached. Most conveniently, the adsorption capacity of the particular adsorption column for the particular wax mixture being separated is determined in advance and the size of the wax charge to the column regulated accordingly. This procedure was followed in this case.

As the wax mixture proceeded down the adsorption column, the olefins were retained by the silica gel and the fully refined paraffinic wax emerged at the bottom. After the entire wax charge had entered the adsorbent, saturating the silica gel with the olefinic wax, the olefinic waxes were desorbed with a suitable eluent, cyclohexanol being employed in this case.

During the initial stages of the desorption

cycle, a mixture of paraffin and olefin waxes containing a higher proportion of olefins than the feed to the column together with cyclohexanol eluent were removed from the bottom of the column and conducted to a stripping column 14 to recover the cyclohexanol eluent for reuse. The paraffin-olefin concentrate, which after one adsorption stage contains in excess of 20% olefins, may be passed to succeeding adsorbers to effect further separation of the olefin and paraffin constituents. If desired, however, the concentrated paraffin olefin wax from the first or from succeeding adsorption stages may be utilized as such.

As the desorption proceeded the paraffin-olefin concentrate was succeeded by a fraction consisting of essentially 100% olefins, herein termed a fully refined olefinic wax. This 100% olefin wax was collected separately.

The fully paraffinic and fully olefinic waxes prepared as above had the following composition:

|                          | Paraffinic Wax | Olefinic Wax |
|--------------------------|----------------|--------------|
|                          | Percent        | Percent      |
| Paraffins and naphthenes | 100            | 0            |
| Olefins                  | 0              | 100          |
| Aromatics                | 0              | 0            |

The fully paraffinic wax had a melting point of 100° to 150° F. and met all the specifications required for a fully refined petroleum paraffin wax. The olefinic wax had a melting point of from 100° to 150° F., was water white, was color stable, and had no objectionable odor or taste.

The fully, or partially olefinic waxes produced in accordance with the invention are unique in that they are high molecular weight materials containing a high degree of olefinic unsaturation. Such unsaturated waxes, which may be produced in large quantities from crude shale oil in accordance with the invention, are difficult to produce synthetically by such methods as the dehydrogenation of paraffin waxes, since the dehydrogenation treatment usually results in degradation of the wax molecule yielding a wax of lower molecular weight.

The olefin waxes produced in accordance with the invention have a melting point ranging between 90° and 200° F. and contain from 20% and up to 100% olefins, principally mono-olefins. The unique properties of these olefinic waxes makes them highly suitable for many applications such as in the production of high melting point halogenated waxes, or as efficient anti-sun checking agents when compounded with rubber (see copending application Ser. No. 247,741 filed September 21, 1951 for Rubber Compound of Improved Resistance to Sun Checking and Other Types of Deterioration by Fred W. Staten). Because of their unsaturated nature these waxes can be readily halogenated.

While the above example illustrates a preferred procedure and preferred conditions for the recovery of olefinic and paraffinic waxes from crude shale oil, it is to be understood that variations in the procedure outlined are possible within the scope of the invention. Thus, for example, the mixture of paraffin and olefin waxes obtained by a single solvent extraction of the wax distillate may be immediately separated into its olefinic and paraffinic constituents without prior treatment to deodorize or decolorize the wax. Similarly solvents and eluents other than those mentioned may be employed. Suitable adsorbents

other than silica gel may be employed to separate the olefins and paraffins, although a silica gel adsorbent is to be preferred for its high adsorbent capacity and adsorbent strength for the olefinic constituents of the wax.

It is to be understood that the above description, together with the specific examples and embodiments described, is intended merely to illustrate the invention, and that the invention is not to be limited thereto, nor in any way except by the scope of the appended claims.

We claim:

1. A method for the recovery of paraffinic and olefinic waxes of relatively high melting point from an oil produced by the destructive distillation of oil shale comprising the steps of solvent extracting a distillation fraction of said shale oil boiling between 675° and 950° F. to recover the waxy material contained therein and then separating the olefinic content of said waxy material from the paraffinic portion thereof to produce one waxy material substantially paraffinic in nature, and another waxy material containing a substantial degree of olefinic unsaturation.

2. A method in accordance with claim 1 in which methylethyl ketone is employed for said solvent extraction.

3. A method for the recovery of paraffinic and olefinic waxes of relatively high melting point from an oil produced by the destructive distillation of oil shale comprising the steps of solvent extracting a distillation fraction of said shale oil boiling between 675° and 950° F. to recover the waxy materials contained therein, contacting the separated waxy material with an adsorbent material to preferentially adsorb the olefinic portion thereof, followed by desorption of the olefinic portion, to produce one waxy material substantially paraffinic in nature, and another waxy material containing a substantial degree of olefinic unsaturation.

4. A method in accordance with claim 3 in which methylethyl ketone is employed for said solvent extraction.

5. A method for the recovery of paraffinic and olefinic waxes of relatively high melting point from an oil produced by the destructive distillation of oil shale comprising the steps of mixing a distillation fraction of said shale oil boiling between 675° and 950° F. with a solvent having substantially no solvent power for the hydrocarbon waxes in said fraction and a strong solvent power for the remaining components of said fraction, reducing said mixture to a temperature of from 0° to 35° F. to permit the hydrocarbon waxes contained in said mixture to be separated therefrom, and then separating the olefinic content of said hydrocarbon waxes from the paraffinic portion thereof to produce one waxy material substantially paraffinic in nature, and another waxy material containing a substantial degree of olefinic unsaturation.

6. A method in accordance with claim 5 in which methylethyl ketone is employed for said solvent extraction.

7. A hydrocarbon wax containing at least 20% of olefinic hydrocarbons and having a melting point above 90° F. obtained by solvent extracting a distillation fraction boiling between 675° and 950° F. of a crude oil obtained by the destructive distillation of oil shale to recover the waxy material herein, and then separating at least a portion of the paraffinic content of said waxy material from the olefinic portion thereof.

8. A hydrocarbon wax consisting of substan-

tially 100% olefinic hydrocarbons and having a melting point above 90° F. obtained by solvent extracting a distillation fraction boiling between 675° and 950° F. of a crude oil obtained by the destructive distillation of oil shale to recover the waxy material contained therein, and then separating the paraffinic content of said waxy material from the olefinic portion thereof.

JOSEPH W. HORNE.  
PETER R. TISOT.

References Cited in the file of this patent

UNITED STATES PATENTS

| Number    | Name            | Date         |
|-----------|-----------------|--------------|
| 2,107,064 | Van der Waerden | Feb. 1, 1938 |

| Number    | Name      | Date          |
|-----------|-----------|---------------|
| 2,459,442 | Lipkin    | Jan. 18, 1949 |
| 2,543,286 | Hirschler | Feb. 27, 1951 |

FOREIGN PATENTS

| Number  | Country       | Date          |
|---------|---------------|---------------|
| 430,485 | Great Britain | June 19, 1935 |

OTHER REFERENCES

10 Warth, The Chemistry and Technology of Waxes, pages 7, 9 and 10, (1947). Reinhold Pub. Co.